# EUROPEAN PATENT SPECIFICATION

(11) **EP 0 830 208 B1**
(45) Date of publication and mention of the grant of the patent: **26.07.2000**
(21) Application number: 96915589.4
(22) Date of filing: 07.05.1996
(51) Int. Cl.: B03D 1/016

(54) **METHOD OF DEPRESSING NON-SULFIDE SILICATE GANGUE MINERALS**
VERFAHREN ZUM DRÜCKEN NICHTSULFIDISCHER SILIKATISCHER GANGARTEN
METHODE DE DEPRESSION DE GANGUES POUR SEPARER DES SILICATES NON SULFURES

(30) Priority: 07.06.1995 US 474805; 07.06.1995 US 475160
(43) Date of publication of application: 25.03.1998
(73) Proprietor: Cytec Technology Corp., Wilmington, Delaware 19801 (US)
(72) Inventor: NAGARAJ, D., R., Stamford, CT 06902 (US); WANG, Samuel, S., Cheshire, CT 06410 (US); LEE, James, S., Sandy Hook, CT 06482 (US); MAGLIOCCO, Lino, Shelton, CT 06484 (US)
(74) Representative: Allam, Peter Clerk
(86) International application number: US9606477
(87) International publication number: WO9640438

(56) References cited:
- AU-B- 502 457
- US-A- 2 740 522
- US-A- 4 220 525
- US-A- 4 360 425
- US-A- 4 720 339
- US-A- 4 744 893
- US-A- 4 902 764

## Description

The present invention relates to froth flotation processes for recovery of value sulfide minerals from base metal sulfide ores. More particularly, it relates to a method for the depression of non-sulfide silicate gangue minerals in the beneficiation of value sulfide minerals by froth flotation procedures.

Certain theory and practice states that the success of a sulfide flotation process depends to a great degree on reagents called collectors that impart selective hydrophobicity to the mineral value which has to be separated from other minerals.

Certain other important reagents, such as the modifiers, are also responsible for the successful flotation separation of the value sulfide and other minerals. Modifiers include, but are not necessarily limited to, all reagents whose principal function is neither collecting nor frothing, but usually one of modifying the surface of the mineral so that it does not float.

In addition to attempts at making sulfide collectors more selective for value sulfide minerals, other approaches to the problem of improving the flotation separation of value sulfide minerals have included the use of modifiers, more particularly depressants, to depress the non-sulfide gangue minerals so that they do not float along with sulfides thereby reducing the levels of non-sulfide gangue minerals reporting to the concentrates. A depressant is a modifier reagent which acts selectively on certain unwanted minerals and prevents or inhibits their flotation.

In sulfide value mineral flotation, certain non-sulfide silicate gangue minerals present a unique problem in that they exhibit natural floatability, i.e. they float independent of the sulfide value mineral collectors used. Even if very selective sulfide value mineral collectors are used, these silicate minerals report to the sulfide concentrates. Talc and pyrophyllite, both belonging to the class of magnesium silicates, are particularly troublesome in that they are naturally highly hydrophobic. Other magnesium silicate minerals belonging to the classes of olivines, pyroxenes, and serpentine exhibit various degrees of floatability that seems to vary from one ore deposit to the other. The presence of these unwanted minerals in sulfide value mineral concentrates causes many problems i.e. a) they increase the mass of the concentrates thus adding to the cost of handling and transportation of the concentrate, b) they compete for space in the froth phase during the flotation stage thereby reducing the overall sulfide value mineral recovery, and c) they dilute the sulfide concentrate with respect to the value sulfide mineral content which makes them less suitable, and in some cases unsuitable, for the smelting thereof because they interfere with the smelting operation.

The depressants commonly used in sulfide flotation include such materials as inorganic salts (NaCN, NaHS, S02, sodium metabisulfite etc) and small amounts of organic compounds such as sodium thioglycolate, mercaptoethanol etc. These depressants are known to be capable of depressing sulfide minerals but are not known to be depressants for non-sulfide minerals, just as known value sulfide collectors are usually not good collectors for non-sulfide value minerals. Sulfide and non-sulfide minerals have vastly different bulk and surface chemical properties. Their response to various chemicals is also vastly different. At present, certain polysaccharides such as guar gum and carboxy methyl cellulose, are used to depress non-sulfide silicate gangue minerals during sulfide flotation. Their performance, however, is very variable and on some ores they show unacceptable depressant activity and the effective dosage per ton of ore is usually very high (as much as 1 to 10 Ibs/ton). Their depressant activity is also influenced by their source and is not consistent from batch to batch. Furthermore, these polysaccharides are also valuable sources of food i.e. their use as depressants reduces their usage as food and, storage thereof presents particular problems with regard to their attractiveness as food for vermin. Lastly, they are not readily miscible or soluble in water and even where water solutions thereof can be made, they are not stable. US-A-4,902,764 (Rothenberg et al.) describes the use of polyacrylamide-based synthetic copolymers and terpolymers for use as sulfide mineral depressants in the recovery of value sulfide minerals. US-A-4,720,339 (Nagaraj et al) describes the use of certain polyacrylamide-based synthetic copolymers and terpolymers, preferably polyacrylamide reacted with glyoxylic acid, as depressants for silicious gangue minerals in the flotation beneficiation of non-sulfide value minerals, but not as depressants in the beneficiation of sulfide value mineral. The '339 patent teaches that such polymers are effective for silica depression during phosphate flotation which also in the flotation stage uses fatty acids and non-sulfide collectors. The patentees do not teach that such polymers are effective depressants for non-sulfide silicate gangue minerals in the recovery of value sulfide minerals.

US-A-4,220,525 (Petrovich) teaches that polyhydroxyamines are useful as depressants for gangue minerals including silica, silicates, carbonates, sulfates and phosphates in the recovery of non-sulfide mineral values. Illustrative examples of the polyhydroxyamines disclosed include aminobutanetriols, aminopartitols, aminohexitols, aminoheptitols, aminooctitols, pentose-amines, hexose amines, amino-tetrols etc. US-A-4,360,425 (Lim et al) describes a method for improving the results of a froth flotation process for the recovery of non-sulfide mineral values wherein a synthetic depressant is added which contains hydroxy and carboxy functionalities. Such depressants are added to the second or amine stage flotation of a double float process for the purpose of depressing non-sulfide value minerals such as phosphate minerals during amine flotation of the siliceous gangue from the second stage concentrate. This patent relates to the use of synthetic depressant during amine flotations only. US-A-2740522 (Aimone et al) teaches that various acrylic polymers, for instance hydrolysed polyacrylonitrile and polyacrylamide, can be used as depressants of siliceous and carbonaceous gangue materials in the flotation of, for instance, sulfide ores. Finally, AU-B-502457 (ICI Australia Limited) discloses that polyvinyl alcohol can be used as depressant in similar flotation processes.

In view of the foregoing and especially in view of the teachings of US-A-4902764 which teaches the use of certain polyacrylamide-based copolymers and terpolymers for sulfide mineral depression during the recovery of value sulfide minerals, we have unexpectedly found that certain polymers, alone or in conjunction with polysaccharides, are indeed excellent depressants for non-sulfide silicate gangue minerals (such as talc, pyroxenes, olivines, serpentine, pyrophyllite, chlorites, biotites, amphiboles, etc) in a froth flotation process for the recovery of value sulfide minerals. These synthetic depressants have now been found to be excellent alternatives to the polysaccharides used currently alone since they, and the blends with polysaccharides, are readily miscible or soluble in water, are non-hazardous and their water solutions are stable. The use thereof will increase the availability of the polysaccharides as a valuable human food source and their performance is not variable. They can be manufactured to adhere to stringent specifications and, accordingly, batch-to-batch consistency is guaranteed. The synthetic polymers lend themselves readily to modification of their structure, thereby permitting tailor-making of depressants for a given application.

In accordance with the present invention there is provided a method for beneficiating value sulfide minerals from ores with the selective rejection of non-sulfide silicate gangue minerals, comprising the steps of:
(a) providing an aqueous pulp slurry of finely-divided, liberation-sized ore particles which contain said value sulfide minerals and said non-sulfide silicate gangue minerals;
(b) conditioning said pulp slurry with an effective amount of non-sulfide silicate gangue mineral depressant, a value sulfide mineral collector and a frothing agent, said depressant comprising either (1) a polymer comprising:
   (i) x units of the formula:
   (ii) y units of the formula:
   (iii) z units of the formula:
   wherein X is the polymerization residue of an acrylamide monomer or mixture of acrylamide monomers, Y is an hydroxy group-containing polymer unit Z is an anionic group-containing polymer unit, x represents a residual mole percent fraction of at least 35%, y is a mole percent fraction ranging from 1 to 50% and z is a mole percent fraction ranging from 0 to 50%, or (2) a mixture of said polymer and a polysaccharide, with the proviso that in case glyoxylated polyacrylamide is used as depressant, it contains less then 50 mole percent glyoxylated amide units as the y units and
c. collecting the value sulfide mineral having a reduced content of non-sulfide silicate gangue minerals by froth flotation.

The polymer depressants of the above formula may comprise, as the (i) units, the polymerization residue of such acrylamides as acrylamide per se and alkyl acrylamides such as methacrylamide and ethacrylamide.

The (ii) units preferably comprise the polymerization residue of monoethylenically unsaturated hydroxyl group containing copolymerization monomers such as hydroxyalkylacrylates and methacrylates e.g. 1,2-dihydroxypropyl acrylate or methacrylate, and hydroxyethyl acrylate or methacrylate; glycidyl methacrylate, acrylamido glycolic acid; hydroxyalkylacrylamides such as N-2-hydroxyethylacrylamide; N-1-hydroxypropylacrylamide, N-bis(1,2-dihydroxyethyl)acrylamide; and N-bis(2-hydroxypropyl)acrylamide.

It is preferred that the (ii) units monomers be incorporated into the polymeric depressant by copolymerization of an appropriate hydroxyl group containing monomer, however, it is also permissible to impart the hydroxyl group substituent to the already polymerized monomer residue by, for example, hydrolysis thereof or post-reaction of a group thereof susceptible to attachment of the desired hydroxyl group with the appropriate reactant material e.g. glyoxal, such as taught in US-A-4,902,764. Glyoxylated polyacrylamide must however, contain less than 50 mole percent glyoxylated amide units, preferably less than 40 mole percent, more preferably less than 30 mole percent, as the Y units. It is preferred that the Y units of the above formula be a non-α-hydroxyl group of the structure wherein A is O or NH, R and R¹ are, individually, hydrogen or a C₁-C₄ alkyl group and n is 1-3, inclusive.

The (iii) units of the polymers useful in the depressants herein may comprise the polymerization residue of an anionic group containing monoethylenically unsaturated, copolymerzable monomer such as acrylic acid, methacrylic acid, alkali metal or ammonium salts of acrylic and/or methacrylic acid, vinyl sulfonate, vinyl phosphonate, 2-acrylamido-2-methyl propane sulfonic acid, styrene sulfonic acid, maleic acid, fumaric acid, crotonic acid, 2-sulfoethylmethacrylate and 2-acrylamido-2-methyl propane phosphonic acid.

Alternatively, but less desirably, the anionic substituents of the (iii) units of the polymers used herein may be imparted thereto by post-reaction such as by hydrolysis of a portion of the (i) unit acrylamide polymerization residue of the polymer as also discussed in the above-mentioned '764 patent.

The effective weight average molecular weight range of these polymers is surprisingly very wide, varying from about a few thousand e.g. 5000, to several millions e.g. 10 million, preferably from about ten thousand to about one million.

The polysaccharides useful as an optional component in the depressant compositions used in the process of the present invention include guar gums; modified guar gums; cellulosics such as carboxymethyl cellulose; and starches. Guar gums are preferred.

If polysaccharide is used, the ratio of the polysaccharide to the polymer in the depressant blend should range from 9:1 to 1:9, respectively, preferably from 7:3 to 3:7, respectively, most preferably from 3:2 to 2:3 respectively.

The dosage of the polymer depressant alone or in combination with the polysaccharide, useful in the method of the present invention, generally ranges from 0.01 to 10 pounds of depressant per ton of ore, preferably from 0.1 to 5 Ib./ton, most preferably from 0.1 to 1.0 lb./ton (1lb.=0.45kg).

The concentration of (i) units in the depressants used herein should be at least 35% as a mole percent fraction of the entire polymer, preferably at least 50%. The concentration of the (ii) units should range from 1 to 50%, as a mole percent fraction, preferably from 5 to 20%, while the concentration of the (iii) units should range from 0 to 50%, as a mole percent fraction, preferably from 1 to 50% and more preferably from 1 to 20%. Mixtures of the polymers composed of the above X, Y and Z units may also be used, for instance in ratios of 9:1 to 1:9.

The new method for beneficiating value sulfide minerals employing the synthetic depressants of the present invention provides excellent metallurgical recovery with improved grade. A wide range of pH and depressant dosage are permissible and compatibility of the depressants with frothers and sulfide value mineral collectors is also an advantage.

The present invention is directed to the selective removal of non-sulfide silicate gangue minerals that normally report to the value sulfide mineral flotation concentrate, either because of natural floatability or hydrophobicity or otherwise. More particularly, the instant method effects the depression of non-sulfide magnesium silicate minerals while enabling the enhanced recovery of sulfide value minerals. Thus, such materials may be treated as, but not limited to, the following:
Talc
Pyrophyllite
Pyroxene group of Minerals
   Diopside
   Augite
   Homeblendes
   Enstatite
   Hypersthene
   Ferrosilite
   Bronzite
Amphibole group of minerals
   Tremolite
   Actinolite
   Anthophyllite
Biotite group of minerals
   Phlogopite
   Biotite
Chlorite group of minerals
Serpentine group of minerals
   Serpentine
   Chrysotile
   Palygorskite
   Lizardite
   Anitgorite
Olivine group of minerals
   Olivine
   Forsterite
   Hortonolite
   Fayalite

The following examples are set forth for purposes of illustration only. All parts and percentages are by weight unless otherwise specified. In the examples, the following designate the monomers used:
AMD = acrylamide
DHPM = 1,2-dihydroxypropyl methacrylate
HEM = 2-hydroxyethyl methacrylate
AA = acrylic acid
MAMD = methacrylamide
VP = vinylphosphonate
GPAM = glyoxylated poly(acrylamide)
APS = 2-acrylamido-2-methylpropane sulfonic acid
VS = vinylsulfonate
CMC = carboxymethyl cellulose
t-BAMD = t-butylacrylamide
HPM = 2-hydroxypropyl methacrylate
HEA = 1-hydroxyethyl acrylate
HPA = 1-hydroxypropyl acrylate
DHPA = 1,2-dihydroxypropyl acrylate
NHE-AMD = N-2-hydroxyethylacrylamide
NHP-AMD = N-2-hydroxypropylacrylamide
NBHE-AMD = N-bis(1,2-dihydroxyethyl)acrylamide
NBEP-AMD = N-bis(1-hydroxypropyl)acrylamide
SEM = 2-sulfethylmethacrylate
AMPP = 2-acrylamido-2-methylpropane phosphonic acid
C = comparative

### Examples 1-41

### Test Procedures

### Pure Talc Flotation

The depressant activity of the polymers is tested using a high grade talc sample in a modified Hallimond tube. 1 Part of talc of size -200+400 mesh is suspended in water and conditioned for 5 min. at the desired pH. A known amount of polymer depressant solution is added and the talc is further conditioned for 5 min. The conditioned talc is then transferred to a flotation cell, and flotation is conducted by passing nitrogen gas for a prescribed length of time. The floated and unfloated talc are then filtered separately, dried and weighed. Percent flotation is then calculated from these weights.

The depressant activity (as measured by % talc flotation; the lower the talc flotation, the greater is the depressant activity) of depressants having varying molecular weights is shown in Table 1. These examples clearly demonstrate that the polymer depressants of the present invention depress talc flotation. In the absence of any polymer, talc flotation is 98%; in the presence of the polymers, talc flotation is in the range of 5 to 58%. The depressant activity, in general, is greater at the high molecular weight. The depressant activity also increases with the proportion of the hydroxy group-containing comonomer.

**Table 1**

| Depressant Concentration: 100 ppm; 8 min. flotation; pH 9 | | |
|---|---|---|
| Example | Depressant | % Talc Flotation |
| 1C | None | 98 |
| 2 | AMD/DHPM, 95/5, MW 10,000 | 31 |
| 3 | AMD/DHPM, 90/10, MW 10,000 | 22 |
| 4 | AMD/DHPM, 80/20, MW 10,000 | 19 |
| 5 | AMD/DHPM, 50/50, MW 10,000 | 20 |
| 6 | AMD/HEM, 95/5, MW 10,000 | 56 |
| 7 | AMD/HEM, 90/10, MW 10,000 | 23 |
| 8 | AMD/DHPM, 90/10, MW 3,000 | 58 |
| 9 | AMD/DHPM, 90/10, MW 10,000 | 32 |
| 10 | AMD/DHPM, 90/10, MW 20,000 | 25 |
| 11 | AMD/DHPM, 90/10, MW 297,000 | 22 |
| 12 | AMD/DHPM, 90/10, MW 397,000 | 5 |
| 13 | AMD/DHPM, 90/10, MW 878,000 | 7 |
| 14 | AMD/HEM, 90/10, MW 3000 | 45 |
| 15 | AMD/HEM, 90/10, MW 10,000 | 12 |
| 16 | AMD/HEM, 90/10, MW 20,000 | 13 |
| 17 | AMD/HEM, 90/10, MW 116,000 | 15 |
| 18 | AMD/HEM, 90/10, MW 286,000 | 20 |
| 19 | AMD/HEM, 90/10, MW 458,000 | 18 |
| 20 | AMD/HEM, 90/10, MW 656,000 | 18 |
| 21 | AMD/DHPM/AA 80/10/10, MW 7000 | 24 |
| 22 | AMD/HEM/AA 80/10/10, MW 8800 | 38 |

The depressant activity at varying dosage of various polymer depressants of the present invention at molecular weights of 10,000 and 300,000 is given in Table 2. In general, the depressant activity increases with the dosage of the polymer. At the high molecular weight, the dosage of the polymer required for a given depression is significantly low.

**Table 2**

| pH 9; 8 min. Flotation | | |
|---|---|---|
| Example | Depressant | % Talc Flotation |
| 23C | None | 98 |
| 24 | AMD/DHPM, 90/10, MW10,000, 5 ppm | 70 |
| 25 | AMD/DHPM, 90/10, MW 10,000, 10 ppm | 59 |
| 26 | AMD/DHPM, 90/10, MW10,000, 40 ppm | 40 |
| 27 | AMD/DHPM, 90/10, MW 10,000, 100 ppm | 21 |
| 28 | AMD/HEM, 90/10, MW10,000, 5 ppm | 52 |
| 29 | AMD/HEM, 90/10, MW 10,000, 10 ppm | 28 |
| 30 | AMD/HEM, 90/10, MW 10,000, 100 ppm | 22 |
| 31 | AMD/DHPM, 90/10, MW 300,000, 1 ppm | 30 |
| 32 | AMD/DHPM, 90/10, MW 300,000, 2.5 ppm | 12 |
| 33 | AMD/DHPM, 90/10, MW 300,000, 100 ppm | 5 |
| 34 | AMD/HEM, 90/10, MW 300,000 1 ppm | 42 |
| 35 | AMD/HEM, 90/10, MW 300,000 10 ppm | 20 |
| 36 | AMD/HEM, 90/10, MW 300,000 100 ppm | 20 |

The depressant activity of a 90/10 acrylamide/dihydroxypropylmethacrylate copolymer at different pH values is given in Table 3. These results demonstrate that the depressant activity is maintained in the wide pH range of 3.5-11.

**Table 3**

| AMD/DHPM 90/10: MW 10,000; DOSAGE 100 PPM; 8 MIN. FLOTATION | | |
|---|---|---|
| NO DEPRESSANT: 95-98% FLOTATION IN THE pH RANGE USED | | |
| Example | pH | % Talc Flotation |
| 37 | 3.5 | 20 |
| 38 | 5 | 35 |
| 39 | 7 | 25 |
| 40 | 9 | 23 |
| 41 | 11 | 26 |

### Examples 42-45

### Natural Sulfide Ore Flotation

### Ore 1

This ore containing approximately 2.25% Ni and 28% MgO (in the form of Mg silicates) is ground in a laboratory rod mill to obtain a pulp at size of 80% -200 mesh. This pulp is transferred to a flotation cell, conditioned at the natural pH (~8.5) with 200 parts/ton of copper sulfate for 4 min., then with 175 parts/ton of sodium ethyl xanthate for 2 min., followed by conditioning with the desired amount of the polymer depressant and an alcohol frother for 1 min. Flotation is then carried out by passing air at approximately 5.5 l/min., and four concentrates are taken. The concentrates and the tails are then filtered, dried and assayed.
The results for two terpolymers depressants of the present invention are compared with those of guar gum in Table 4. The objective here is to decrease the Mg-silicate recovery (as identified by MgO as an indicator) into the sulfide flotation concentrate while maintaining as high a Ni recovery and Ni grade as possible. The results in Table 4 demonstrate that the two terpolymer depressants of the present invention provided about 3 units lower MgO recovery while providing equal of slightly better Ni recovery and Ni grade at only 75% of the guar gum dosage. In the absence of any depressant, the MgO recovery is much higher (27%) which is unacceptable.

**Table 4**

| Feed Assay: 2.25% Ni and 27.7 MgO | | | | | | |
|---|---|---|---|---|---|---|
| Example | Depressant | p/t | Cum. Wt.%. C1-4 | Ni Rec. | Ni Grade | MgO Rec. |
| 42C | None | 0 | 36.87 | 80.5 | 5.0 | 27.0 |
| 43C | Guar Gum | 175 | 31.10 | 76.1 | 5.4 | 21.5 |
| 44 | AMD/DHPM/AA 80/10/10, 7K | 130 | 27.88 | 77.6 | 6.4 | 18.6 |
| 45 | AMD/HEM/AA 80/10/10, 9K | 130 | 26.98 | 75.1 | 6.3 | 18.5 |

### Examples 46-54 and 56-65

### Ore 2

This ore containing approximately 3.3% Ni and 17.6% MgO (in the form of Mg silicates) is ground in a laboratory rod mill for 5 min. to obtain a pulp at a size of 81% -200 mesh. The ground pulp is then transferred to a flotation cell, and is conditioned at the natural pH (~8-8.5) with 150 parts/ton of copper sulfate for 2 min., 50 to 100 parts/ton of sodium ethyl xanthate for 2 min. and then with the desired amount of a depressant and an alcohol for 2 min. First stage flotation is then conducted by passing air at approximately 3.5-5 l/min. and a concentrate is collected. In the second stage, the pulp is conditioned with 10 parts/ton of sodium ethyl xanthate, and desired amounts of the depressant and the frother for 2 min. and a concentrate is collected. The conditions used in the second stage are also used in the third stage and a concentrate is collected. All of the flotation products are filtered, dried and assayed.

In Table 5 (in which there is no Example 55), the depressant activity of several copolymer and terpolymer depressants is compared with that of guar gum at two different dosages. In the absence of any depressant, the Ni recovery is 96.6% which is considered very high and desirable; the MgO recovery is 61.4% which is also very high, but considered highly undesirable. The Ni grade of 4.7% obtained is only slightly higher than that in the original feed. With guar gum at 420 and 500 parts/ton, the MgO recovery is in the range of 28.3 to 33.5% which is considerably lower than that obtained in the absence of a depressant, and Ni recovery is about 93% which is lower than that obtained in the absence of depressant. A reduction in Ni recovery is to be expected in the process of reducing MgO recovery since there is invariably some mineralogical association of Ni minerals with the Mg-silicates; when the latter are depressed, some Ni minerals are also depressed. The synthetic polymer depressants of the present invention show much stronger depressant activity than guar gum; the MgO recoveries are in the range of 6.3 to 15.3% compared with 28.3-33-5% for guar gum. These results indicate that significantly lower dosage of the synthetic depressants can be used if results similar to those of guar gum are desired. The terpolymer containing 10 parts each of methacrylamide and dihydroxypropyl methacrylate provides depressant activity that is similar to that of guar gum. Similarly, a terpolymer of AMD, DHPM and vinyl phosphonate provides metallurgy that is similar to guar gum.

It is pertinent to note here that polyacrylamide reacted with glyoxylic acid, containing pendant hydroxyl and carboxyl groups, shows depressant activity at a degree of substitution of 10% (i.e. 10 parts of the amide groups in the polyacrylamide are reacted with glyoxylic acid.) At a degree of substitution of 50%, depressant activity is weaker.

**Table 5**

| Feed Assay: 3.31% Ni and 17.58% MgO | | | | | |
|---|---|---|---|---|---|
| Example | Depressant | p/t | Ni Rec. | Ni Grade | MgO Rec. |
| 46C | None | 0 | 96.6 | 4.7 | 61.4 |
| 47C | Guar Gum | 350+70+80 | 93.0 | 7.7 | 28.3 |
| 48C | Guar Gum | 300+60+60 | 92.9 | 6.7 | 33.5 |
| 49 | AMD/DHPM 90/10, 397K | 350+60+60 | 84.5 | 10.5 | 12.6 |
| 50 | AMD/DHPM 90/10, 878K | 350+70+80 | 81.8 | 12.6 | 8.2 |
| 51 | AMD/DHPM 90/10, 878K | 280+56+64 | 84.2 | 8.0 | 15.3 |
| 52 | AMD/DHPM 80/20, 500K | 350+70+80 | 80.3 | 11.5 | 9.8 |
| 53 | AMD/DHPM 80/20, 800K | 350+70+80 | 71.4 | 11.8 | 6.3 |
| 54 | AMD/MAMD/DHPM 80/10/10, 6.23K | 350+85+ 100 | 92.3 | 7.2 | 37.6 |
| 56 | GPAM (90/10) | 350+70+80 | 93.3 | 6.3 | 43.7 |
| 57C | GPAM (50/50) | 350+70+80 | 99.0 | 4.7 | 63.4 |
| 58 | AMD/HPM 90/10 | 350+85+ 100 | 94.6 | 6.4 | 44.0 |
| 59 | AMD/HEM 90/10, 656K | 250+60+70 | 86.4 | 7.0 | 27.9 |
| 60 | AMD/DHPM/HEM 95/5/5 | 280+56+64 | 84.1 | 6.9 | 23.9 |
| 61 | AMD/DHPM/AA 80/10/10, 750K | 250+60+70 | 91.8 | 5.6 | 39.2 |
| 62 | -do- | 280+56+64 | 89.6 | 6.2 | 28.1 |
| 63 | AMD/DHPM/AA 85/10/5, 800K | -do- | 89.6 | 7.2 | 24.6 |
| 64 | AMD/DHPM/APS 80/10/10, 11.7K | 250+60+70 | 95.0 | 6.5 | 47.5 |
| 65 | AMD/DHPMNS 80/10/10, 7.78K | -do- | 94.1 | 7.0 | 42.9 |
| 65A | Polymer of Examples 59 and 61 in a ratio of 1:1 | 350+70+80 | 92.5 | 10.3 | 16.8 |

### Examples 66-79

### Ore 3

This ore has approximately 2.1% Ni and 17% MgO. 1000 Parts of ore is ground in a rod mill to obtain a pulp that has a size of 80% passing 20 mesh. The ground pulp is conditioned for 2 min. with 200 parts/ton of copper sulfate, 2 min. with 100 parts/ton of sodium ethyl xanthate and the required amount of frother, and then for 2 min. with the desired amount of the depressant. Flotation is then conducted by passing air, and a concentrate is taken. In the second stage, the pulp is conditioned with 40 parts/ton of xanthate and additional amounts of the same depressant, and a second concentrate is taken. A third stage flotation is conducted similarly and a concentrate is taken. All of the flotation products are filtered, dried and assayed.

The results for the depressant activity of several of the synthetic copolymer and terpolymer depressants of the present invention are compared with that of guar gum (at two dosages) in Table 6. These results demonstrate clearly that the depressants provide metallurgy that is equal or better than that of guar gum at 40 to 70% of the guar gum dosage. In many examples, improved Ni recovery is obtained while maintaining a low MgO recovery indicating gangue silicate mineral depression.

**Table 6**

| Feed Assay: Ni 2.06%; MgO 17% - Xanthate Rougher Float | | | | | | |
|---|---|---|---|---|---|---|
| | | Dose | Cum. | Grade | Cum. Rec. % | |
| Example | Depressant | p/t | Wt.% | Ni | Ni | MgO |
| 66C | GUAR | 200 | 27.9 | 6.11 | 84.6 | 13.1 |
| 67C | GUAR | 250 | 27.0 | 6.31 | 84.4 | 12.1 |
| 68 | AMD/DHPM 90/10, 397K | 100 | 29.4 | 6.20 | 86.6 | 13.5 |
| 69 | AMD/DHPM 90/10, 397K | 140 | 27.5 | 6.29 | 85.6 | 12.7 |
| 70 | AMD/DHPM 90/10, 878K | 100 | 28.0 | 6.45 | 85.6 | 12.5 |
| 71 | AMD/DHPM 90/10, 878K | 180 | 28.3 | 6.39 | 84.8 | 12.8 |
| 72 | AMD/HEM 90/10, 286K | 140 | 27.9 | 6.22 | 85.1 | 12.8 |
| 73 | AMD/HEM 90/10, 286K | 180 | 26.7 | 6.66 | 84.4 | 10.9 |
| 74 | AMD/HEM 90/10, 656K | 100 | 27.9 | 6.54 | 85.2 | 12.1 |
| 75 | AMD/HEM 90/10, 656K | 180 | 26.6 | 6.50 | 83.7 | 11.2 |
| 76 | AMD/DHPM/AA 80/10/10, 750K | 140 | 28.3 | 6.15 | 84.5 | 12.6 |
| 77 | AMD/DHPM/AA 80/10/10, 750K | 180 | 27.8 | 6.48 | 85.4 | 12.4 |
| 78 | AMD/HEM/AA 80/10/10, 224K | 140 | 28.9 | 6.18 | 86.0 | 13.8 |
| 79 | AMD/HEM/AA 80/10/10, 224K | 180 | 27.4 | 6.33 | 84.2 | 12.5 |

### Examples 80-83

### Ore 4

This ore containing approximately 0.6% Ni and about 38% MgO (in the form of Mg silicates) is ground in a laboratory rod mill to obtain a pulp at a size of 80% -200 mesh. This ground pulp is deslimed, conditioned for 20 min. with 120 parts/ton of sodium ethyl xanthate and the desired amount of frother. Flotation is then conducted and a concentrate is collected for 4 min. This concentrate is then conditioned for 1 min. with 20 parts/ton of sodium ethyl xanthate and with the specified amount of the depressant. A cleaner flotation is then carried out for 3.5 min. The concentrate and tails are then filtered, dried and assayed.

The results for the depressant activity of three synthetic polymer depressants are compared with that of guar gum in Table 7. It is again evident from the results in Table 7 that the synthetic depressants of this invention provide metallurgy that is equal to or better than guar gum at 40 to 80% of the guar dosage. With two of the depressants the Ni recovery is significantly improved while maintaining low MgO recoveries.

**Table 7**

| Example | Depressant | Dose (p/t) | Cum. Wt.% | Grade | Cum. Recovery | |
|---|---|---|---|---|---|---|
| | | | | Ni | Ni | MgO |
| 80C | Guar | 30 | 3.8 | 9.2 | 62.6 | 2.3 |
| 81 | AMD/DHPM 90/10, 397K | 15 | 4.4 | 9.1 | 65.8 | 2.6 |
| 82 | AMD/DHPM 90/10, 397K | 12.5 | 4.7 | 7.5 | 66.2 | 3.0 |
| 83 | AMD/HEM/AA 80/10/10, 224K | 24 | 3.8 | 9.0 | 61.7 | 2.4 |

### Examples 84-96

### Ore 5

This ore containing small amounts of Ni, Cu and Fe in the form of sulfides, small amounts of platinum and palladium, and approximately 7.5% MgO (in the form of Mg silicates) is ground in a laboratory rod mill with 15 parts/ton of potassium amyl xanthate and 12.5 parts/ton of diisobutyl dithiophosphate for 10 min. to obtain a pulp at a size of 40% - 200 mesh. The ground pulp is then transferred to a flotation cell, and is conditioned for 2 min. at the natural pH (~8.2) with the same amounts of collectors as in the grind, followed by conditioning with the specified amount of depressant and an alcohol frother for 2 min. Flotation is then conducted by passing approximately 3.5-5 Vmin. of air and a concentrate is collected. The procedure used in the first stage of flotation is followed in the second stage and a second concentrate is collected. The flotation products are then filtered, dried and assayed.

The results for the depressant activity of a variety of synthetic polymer depressants of the present invention are compared in Table 8 with that of two carboxy methyl cellulose samples from different sources. The objective here is to obtain high recovery and grades of Pt and Pd in the concentrate. In the absence of any depressant, the recovery of Pt and Pd is indeed very high (97.5% and 94-95% respectively), but the concentrate grades are unacceptably low. With the CMC depressants, the Pt and Pd recoveries are 95-96.5% and 92-94.6%, respectively, and the grades are 3-3.1 for Pt and 12.7-13 for Pd. It is evident from the results that the synthetic polymer depressants provide Pt and Pd metallurgy that is equal to or better than that of CMC samples and at significantly lower dosages (60-80% of the CMC dosage). It is also evident that the synthetic polymer depressants provide better grades for the Pt which is a more important and much higher value metal than Pd. In Example 88, a polymer containing only 0.5 part of the t-butyl acrylamide in addition to DHPM provides Pt metallurgy that is equal to that of CMC(B) but at 80% of the dosage of CMC.

**Table 8**

| Feed Assay: 5.8 p/t Pt; 22 p/t Pd | | | | | | |
|---|---|---|---|---|---|---|
| Example | Depressant | p/t | Pt Rec. | Pt Grade | Pd Rec. | Pd Grade |
| 84C | None | 0 | 97.5 | 1.6 | 95.0 | 6.0 |
| 85C | None | 0 | 97.6 | 2.3 | 94.4 | 72 |
| 86C | CMC-A | 500 | 95.2 | 3.1 | 92.0 | 12.7 |
| 87C | CMC-B | 500 | 96.5 | 3.0 | 94.6 | 13.0 |
| 88 | AMD/DHPM/t-BAMD 89.5/10/0.5 | 400 | 96.5 | 3.1 | 93.1 | 11.6 |
| 89 | AMD/DHPM/AA 80/10/10, 750K | 400 | 96.6 | 2.1 | 93.2 | 7.4 |
| 90 | AMD/DHPM/AA 80/10/10, 750K | 500 | 92.9 | 4.6 | 88.3 | 14.7 |
| 91 | AMD/HEM/AA 80/10/10. 224K | 370 | 94.5 | 3.8 | 92.1 | 13.9 |
| 92 | AMD/HEM/AA 80/10/10, 224K | 300 | 95.3 | 42 | 91.4 | 16.4 |
| 93 | AMD/HEM/AA 80/10/10, 224K | 400 | 96.6 | 2.7 | 94.1 | 10.6 |
| 94 | AMD/DHPM/AA 85/10/5 | 400 | 96.8 | 32 | 93.4 | 11.2 |
| 95 | AMD/DHPM/VP 80/10/10, 12K | 370 | 96.9 | 2.8 | 94.1 | 10.4 |
| 96 | AMD/DHPM/MAMD 80/10/10 | 400 | 94.8 | 1.6 | 91.9 | 6.5 |

### Examples 97-99

### Ore 6

This ore contains 0.85% Ni and 39% MgO. 1000 Parts of the ore are ground in a rod mill to give a flotation feed of size 80% passing 200 mesh. The ground pulp is conditioned for 30 min. with the desired amount of a depressant along with 500 parts/ton sodium ethyl xanthate. Rougher flotation is then carried out for 25 min. The rougher concentrate is then conditioned with the specified amount of depressant and 10 parts/ton of sodium ethyl xanthate and a cleaner flotation is carried out for 15 min. The flotation products are filtered, dried and assayed.

The results for two synthetic copolymers of AMD/DHPM are compared with that of CMC in Table 9. These results demonstrate that the synthetic depressants provide metallurgy that is equal to or better than that of CMC, but at about 27% of the CMC dosage. In the case of the copolymer with a molecular weight of 878,000, the MgO recovery in both the regular and cleaner concentrate is significantly lower than that obtained with CMC.

**Table 9**

| Feed Assay: Ni 0.85%; MgO 39% | | | | | | | |
|---|---|---|---|---|---|---|---|
| Example | Depressant | Dose p/t Total | Product | Grade Ni | Cum. Recovery, % | | |
| | | | | | Wt | Ni | MgO |
| 97C | CMC | 275 | 1ClCon | 15.44 | 3.48 | 60.8 | 2.3 |
| | | | RoCon | 3.21 | 21.17 | 76.8 | 20.6 |
| 98 | AMD/DHPM 90/10, 878K | 75 | 1CICon | 18.01 | 2.73 | 59.3 | 1.5 |
| | | | RoCon | 3.78 | 15.92 | 72.6 | 14.6 |
| 99 | AMD/DHPM 90/10, 397K | 75 | 1CICon | 14.48 | 3.41 | 61.6 | 2.1 |
| | | | RoCon | 2.83 | 21.96 | 77.6 | 20.7 |

### Examples 100-109

### Ore 7

This ore containing small amounts of Ni, Cu, and Fe in form of sulfides and about 17% MgO (in the form of Mg silicates) is ground in a laboratory ball mill for 12 min. to obtain a pulp at a size of 40% -200 mesh. The ground pulp is then transferred to a flotation cell, and is conditioned at the natural pH (~7.2) with the specified amount of a depressant for 3 min., followed with 16 parts/ton of sodium isobutyl xanthate and 34 parts/ton of a dithiophosphate and a polyglycol frother for 3 min. Flotation is then conducted by passing air at approximately 3.5 Vmin. and two concentrates are collected. The flotation products are then filtered, dried and assayed.

The results for the depressant activity of a variety of synthetic polymer depressants of the present invention are compared with that of a modified guar in Table 10. The objection here is to minimize the recovery of SiO2, CaO, MgO, Al203 - all of which represent the silicate minerals present in the sulfide concentrates - and to maintain or improve the recovery of Ni and Cu which constitute the value sulfide minerals. In the absence of any depressant, the Ni and Cu recoveries are 49.5% and 79%, respectively, but the recovery of the gangue constituents is very high (9.4% for SiO2, 7.4% for CaO, 10.6% for MgO and 5.8% for Al203). With guar, both the Ni and Cu recoveries are slightly reduced, perhaps because of depression of some silicate minerals that carry Ni and Cu sulfides as mineral locking, but recovery of the gangue constituents is also reduced. With all of the synthetic polymer depressants tested, there is a significant reduction in the recovery of the gangue constituents, and with some of them the reduction is far greater than that obtained with guar. All of the depressants of the present invention (except one) give higher copper recoveries than guar; in some cases the copper recoveries are higher than that obtained in the absence of the depressant. Also the Ni recoveries obtained with the synthetic depressants are either equal to or much greater than that obtained with guar. In the best case, AMD/HEM 90/10, 10,000 MW, there is more than 50% reduction in SiO2 compared to the test with no depressant, and 44% reduction in SiO2 compared to that with guar. Similarly significant reductions are also observed for other gangue constituents.

**Table 10**

| Calculated Head Assays: Cu - 0.07%, Ni - 0.20%; SiO2 - 48.8%; CaO - 5.8% MgO - 17%; Al203 - 9% | | | | | | | | | |
|---|---|---|---|---|---|---|---|---|---|
| Example | Depressant | p/t | Order of Addn. | Copper | Nickel | Si02 | CaO | MgO | A1203 |
| | | | | Rec | Rec | Rec | Rec | Rec | Rec |
| 100C | None | 0 | - | 79.0 | 49.5 | 9.4 | 7.4 | 10.6 | 5.8 |
| 101C | Guar | 60 | Depr 1st | 77.2 | 46.2 | 7.5 | 5.9 | 8.6 | 4.8 |
| 102 | AMD/HEM 95/5 100k | 60 | Depr 1st | 75.9 | 46.3 | 8.5 | 6.8 | 9.5 | 5.6 |
| 103 | AMD/HEM 90/10 20k | 60 | Depr 1st | 78.3 | 48.6 | 8.0 | 6.4 | 9.2 | 5.2 |
| 104 | AMD/HEM 90/10 10k | 70 | Depr Ist | 81.3 | 51.0 | 7.3 | 5.9 | 8.2 | 4.9 |
| 105 | AMD/HEM 90/10 10k | 70 | Reverse | 82.4 | 50.1 | 4.2 | 5.1 | 7.5 | 3.9 |
| 106 | AMD/DHPM 80/20 10k | 67 | Depr 1st | 79.4 | 46.5 | 6.5 | 4.9 | 7.4 | 3.8 |
| 107 | AMD/DHPM 90/10 10k | 60 | Depr 1st | 79.3 | 48.2 | 7.4 | 5.9 | 8.5 | 4.7 |
| 108 | AMD/DHPM 90/10 10k | 60 | Reverse | 80.2 | 47.5 | 6.5 | 5.0 | 7.5 | 4.0 |
| 109 | AMD/DHPM/AA 80/10/10 10k | 60 | Depr 1st | 78.4 | 46.3 | 72 | 5.9 | 8.2 | 4.9 |

### Example 110

Following the procedure of Example 50 except that the DHPM is replaced by an equivalent amount of HEA, similar results are obtained.

### Example 111

Replacing the HEM of Example 45 with DHPA achieves substantially similar results.

### Examples 112

Example 53 is again followed but the DHPM is replaced by HPA to achieve similar recovery.

### Example 113

When the HEM of Example 73 is replaced by NHE-AMD similar cumulative recovery of nickel and magnesium is observed.

### Example 114

NBHE-AMD is used to replace DHPM in the Example 88 procedure. The results are similar.

### Example 115

The DHPM of Example 96 is replaced by NHP-AMD to yield similar platinum and palladium recoveries.

### Example 116

Metal recoveries are similar when the HEM of Example 102 is replaced by NBEP-AMD.

### Example 117

Replacement of the AA of Example 22 by SEM results in similar % talc flotation.

### Example 118

When the VP of Example 55 is replaced by AMPP, similar results are achieved.

### Examples 119-127

An ore containing approximately 3.3% Ni and 16.5% MgO (in the form of Mg silicates) is ground in a laboratory rod mill for 5 minutes to obtain a pulp at a size of 81% - 200 mesh. The ground pulp is then transferred to a flotation cell, and is conditioned at the natural pH (~8-8.5) with 150 parts/ton of copper sulfate for 2 minutes, 50 to 100 parts/ton of sodium ethyl xanthate for 2 minutes and then with the desired amount of depressant blend and an alcohol frother for 2 minutes. First stage flotation is then conducted by passing air at approximately 3.5-5 l/min. and a concentrate is collected. In the second stage, the pulp is conditioned with 10 parts/ton of sodium ethyl xanthate, and desired amounts of depressant blend and the frother for 2 minutes and a concentrate is collected. The conditions used in the second stage are also used in the third stage and a concentrate is collected. All of the flotation products are filtered, dried and assayed.

The depressant activity of a 1:1 blend of AMD/DHPM and guar gum is compared with the individual depressants in Table II. With guar alone the Ni recovery is 93% and MgO recovery is 28.3%. With the synthetic polymer depressant alone, the Ni recovery is 84.5% and the MgO recovery is 12.6% which is less than half of that of guar gum, thereby indicating a very strong depressant activity of the synthetic depressant. In the case of the blend, there is a further reduction in MgO recovery and the Ni recovery and grade improve slightly over that of the synthetic depressant. These results demonstrate the greater depressant activity obtained with the blend and also suggest that much lower dosages can be used compared to those of the individual components.

The depressant activity of a 1:1 blend of AMD/HEM polymer and guar gum is compared with that of the individual depressants in Table 2. With guar gum alone, as before, the Ni recovery is 93% and the MgO recovery is 28.3%. With the AMD/HEM copolymer at the same dosage, the MgO recovery is only 7.7% indicating a very strong depressant activity; the Ni recovery is also significantly reduced (68.3% vs. 93% for guar). With the blend, however, the Ni recovery improves significantly (82.8%) while the MgO recovery is maintained at the low level of 8.3%. The results also suggest that a considerably lower dosage can be used with the blend to obtain enhanced performance. In fact, when the dosage is lowered to 430 parts/ton, the Ni recovery increases to 86% (from 82.8%) while the MgO recovery increases to 11.5% (from 8.3%).

**Table II**

| FEED ASSAY: 3.31% Ni and 17.58% MgO | | | | | |
|---|---|---|---|---|---|
| Example | Depressant | g/t | Ni Rec | Ni Grade | Mgo Rec. |
| 119C | None | 0 | 96.6 | 4.7 | 61.4 |
| 120C | Guar Gum | 350+70+80 | 93.0 | 7.7 | 28.3 |
| 121C | AMD/DHPM 90/10; 397K | 300+60+60 | 84.5 | 10.5 | 12.6 |
| 122 | Guar Gum and AMD/DHPM 1:1 90/10; 397K | 350+70+80 | 85.7 | 11.0 | 10.3 |
| 123C | None | 0 | 96.6 | 4.7 | 61.4 |
| 124C | Guar Gum | 350+70+80 | 93.0 | 7.7 | 28.3 |
| 125C | AMD/HEM 90/10; 656K | 350+70+80 | 68.3 | 11.4 | 7.7 |
| 126 | Guar Gum and AMD/HEM 1:1 90/10; 656K | 300+70+80 | 82.8 | 12.2 | 8.3 |
| 127 | Guar Gum and AMD/HEM 1:1 90/10; 656K | 30+60+70 | 86.0 | 10.3 | 11.5 |

### Examples 128-143

When the procedures of Examples 119-127 are again followed except that the depressant components are varied, as are their concentrations, as set forth in Table 12, below, similar results are achieved.

**Table 12**

| Example | Polymer (PM) | Polysaccharide (PS) | PM:PS Ratio |
|---|---|---|---|
| 128 | AMD/MAMD/DHPM 80/10/10; 623K | Guar Gum | 9:1 |
| 129 | AMD/DHPM/AA 80/10/10; 7K | Starch | 1:1 |
| 130 | -do- 750K | CMC | 4:1 |
| 131 | AMD/MAMDNP 80/10/10; 12K | Modified Guar | 2:3 |
| 132 | GPAM (90/10) | -do- | 1:4 |
| 133 | AMD/HEM/AA 80/10/10; 9K | CMC | 1:1 |
| 134 | AMD/HEM/t-BAMD 89.5/10/0.5 | Guar Gum | 1:9 |
| 135 | AMD/DHPM/APS 80/10/10; 11.7K | Starch | 2:1 |
| 136 | AMD/DHPM/VS 80/10/10; 7.78K | Guar Gum | 3:2 |
| 137 | AMD/HPA 80/20 | Guar Gum | 1:1 |
| 138 | AMD/DHPA/AA 80/10/10 | Guar Gum | 1:1 |
| 139 | AMD/NHE-AMD 90/10 | CMC | 1:1 |
| 140 | AMD/NBHE-AMD/BAMD 89.5/10/0.5 | Starch | 1:1 |
| 141 | AMD/NHP-AMD/MAMD 80/10/10 | Guar Gum | 1:1 |
| 142 | AMD/NBEP-AMD 95/5 | Guar Gum | 1:1 |
| 143 | AMD/HEM/SEM 80/10/10 | Guar Gum | 1:1 |

## Claims

1. A method for beneficiating value sulfide minerals from ores with selective rejection of non-sulfide silicate gangue minerals comprising the steps of:
a. providing an aqueous pulp slurry of finely-divided, liberation-sized ore particles which contain said value sulfide minerals and said non-sulfide silicate gangue minerals;
b. conditioning said pulp slurry with an effective amount of non-sulfide silicate gangue mineral depressant, a value sulfide mineral collector and a frothing agent, respectively, said depressant comprising either (1) a polymer or a mixture of polymers comprising:
(i) x units of the formula:
⁅X⁆
(ii) y units of the formula
⁅Y⁆
(iii) z units of the formula:
⁅Z⁆
wherein X is the polymerization residue of an acrylamide monomer or mixture of acrylamide monomers, Y is an hydroxy group containing polymer unit, Z is an anionic group containing polymer unit, x represents a residual mole percent fraction of at least 35%, y is a mole percent fraction ranging from 1 to 50% and z is a mole percent fraction ranging from 0 to 50% or (2) a mixture of said polymer or polymers and a polysaccharide, with the proviso that in case glyoxylated polyacrylamide is used as depressant, it contains less than 50 mole percent glyoxylated amide units as the y units, and
c. collecting the value sulfide mineral having a reduced content of non-sulfide silicate gangue minerals by froth flotation.

2. A method according to Claim 1, wherein Y has the formula wherein A is O or NH, R and R¹ are, individually, hydrogen or a C₁ - C₄ alkyl group and n is 1-3, inclusive.

3. A method according to Claim 1, wherein X is the polymerization residue of acrylamide, Y is the polymerization residue of 1,2-dihydroxypropyl methacrylate and z is 0.

4. A method according to Claim 1, wherein X is the polymerization residue of acrylamide, Y is the polymerization residue of 1, 2-dihydroxypropyl methacrylate, Z is the polymerization residue of acrylic acid and z is a mole percent fraction ranging from 1 to 50.

5. A method according to Claim 1, wherein X is the polymerization residue of acrylamide, Y is the polymerization residue of hydroxyethyl methacrylate and z is 0.

6. A method according to Claim 1, wherein X is the polymerization residue of acrylamide, Y is the polymerization residue of hydroxyethyl methacrylate, Z is the polymerization residue of acrylic acid and z is a mole percent fraction ranging from 1 to 50%.

7. A method according to Claim 1, wherein X is the polymerization residue of acrylamide, Y is the polymerization residue of 1,2-dihydroxypropyl methacrylate, Z is the polymerization residue of vinyl sulfonate and z is a mole percent fraction ranging from 1 to 50%.

8. A method according to Claim 1, wherein X is the polymerization residue of acrylamide, Y is the polymerization residue of 1,2-dihydroxypropyl methacrylate, Z is the polymerization residue of vinyl phosphonate and z is a mole percent fraction ranging from 1 to 50%.

9. A method according to Claim 1 wherein X is the polymerization residue of acrylamide, Y is the polymerization residue of hydroxyethyl methacrylate, Z is the polymerization residue of vinyl sulfonate and z is a mole percent fraction ranging from 1 to 50%.

10. A method according to Claim 1, wherein X is the polymerization residue of acrylamide, Y is the polymerization residue of hydroxyethyl methacrylate, Z is the polymerization residue of vinyl phosphonate and z is a mole percent fraction ranging from 1 to 50%.

11. A method according to Claim 1, wherein X is the polymerization residue of acrylamide, Y is the polymerization residue of 1, 2-dihydroxypropyl methacrylate, Z is the polymerization residue of 2-acrylamido-2-methyl propane sulfonic acid and z is a mole percent fraction ranging from 1 to 50.

12. A method according to Claim 1, wherein X is the polymerization residue of acrylamide, Y is the polymerization residue of hydroxyethyl methacrylate, Z is the polymerization residue of 2-acrylamido-2-methyl propane sulfonic acid and z is a mole percent fraction ranging from 1 to 50%.

13. A method according to Claim 1, wherein X is the polymerization residue of acrylamide and t-butylacrylamide, Y is the polymerization residue of 1,2-dihydroxypropyl methacrylate and z is 0.

14. A method according to Claim 1, wherein X is the polymerization residue of acrylamide, and methacrylamide, Y is the polymerization residue of 1,2-dihydroxypropyl methacrylate and z is 0.

15. A method according to Claim 1, wherein X is the polymerization residue of acrylamide and methacrylamide, Y is the polymerization residue of hydroxyethyl methacrylate and z is 0.

16. A method according to Claim 1, wherein Y represents a glyoxylated acrylamide unit and y is less than about 40.

17. A method according to Claim 1, wherein X is the polymerization residue of acrylamide and t-butylacrylamide, Y is the polymerization residue of hydroxyethyl methacrylate and z is O.

18. A method according to any preceding Claim, wherein the polysaccharide is guar gum.

19. A method according to any one of Claims 1-17, wherein the polysaccharide is carboxymethyl cellulose.

20. A method according to any one of Claims 1-17, wherein the polysaccharide is starch.

## Patentansprüche

1. Verfahren zur Aufbereitung von nutzbaren Sulfidmineralien aus Erzen bei selektiver Zurückweisung von nichtsulfidischen Silikat-Gangmineralien, welches die folgenden Schritte umfaßt:
a. Schaffen einer wäßrigen Aufschlämmung aus feinverteilten, Aufschluß-dimensionierten Erzteilchen, welche die nutzbaren Sulfidmineralien und die nichtsulfidischen Silikaten-Gangmineralien enthält;
b. Behandeln der wäßrigen Aufschlämmung mit einer wirksamen Menge eines Sinkmittels für nichtsulfidische Silikat-Gangmineralien, eines Abscheiders für nutzbare Sulfidmineralien beziehungsweise eines Schaumbildners, wobei das Sinkmittel umfaßt: entweder (1) ein Polymer oder eine Polymermischung, die folgendes umfaßt:
(i) x Einheiten mit der Formel:
⁅X⁆
(ii) y Einheiten mit der Formel:
⁅Y⁆
(iii) z Einheiten mit der Formel:
⁅Z⁆
wobei X das Polymerisationsradikal eines Acrylamid-Monomers oder einer Acrylamid-Monomermischung ist, Y eine Polymereinheit ist, welche eine Hydroxygruppe enthält, Z eine Polymereinheit ist, welche eine anionische Gruppe enthält, x einen molaren Restanteil von zumindest 35 % darstellt, y ein molarer Anteil ist, welcher sich von 1 bis 50 % erstreckt, und z ein molarer Anteil ist, welcher sich von 0 bis 50 % erstreckt, oder (2) eine Mischung des Polymers oder Polymere und ein Polysaccharid, unter der Bedingung, daß sie bei Verwendung von glyoxyliertem Polyacrylamid als Sinkmittel weniger als 50 Molprozent glyoxylierte Amid-Einheiten als Y-Einheiten enthält, und
c. Abscheiden der nutzbaren Sulfidmineralien, die durch Schaumflotation einen verringerten Gehalt an nichtsulfidischen Silikat-Gangmineralien aufweisen.

2. Verfahren nach Anspruch 1, wobei Y die Formel aufweist, wobei A O oder NH ist, R und R¹ jedes für sich Wasserstoff oder eine C₁-C₄-Alkylgruppe ist und n = 1 bis einschließlich 3 ist.

3. Verfahren nach Anspruch 1, wobei X das Polymerisationsradikal von Acrylamid ist, Y das Polymerisationsradikal von 1,2-Dihydroxypropyl-Methacrylat ist und z = 0 ist.

4. Verfahren nach Anspruch 1, wobei X das Polymerisationsradikal von Acrylamid ist, Y das Polymerisationsradikal von 1,2-Dihydroxypropyl-Methacrylat ist, Z das Polymerisationsradikal von Acrylsäure ist und z ein molarer Prozentanteil im Bereich von 1 bis 50 ist.

5. Verfahren nach Anspruch 1, wobei X das Polymerisationsradikal von Acrylamid ist, Y das Polymerisationsradikal von Hydroxyethyl-Methacrylat ist und z = 0 ist.

6. Verfahren nach Anspruch 1, wobei X das Polymerisationsradikal von Acrylamid ist, Y das Polymerisationsradikal von Hydroxyethyl-Methacrylat ist, Z das Polymerisationsradikal von Acrylsäure ist und z ein molarer Prozentanteil im Bereich von 1 bis 50 % ist.

7. Verfahren nach Anspruch 1, wobei X das Polymerisationsradikal von Acrylamid ist, Y das Polymerisationsradikal von 1,2-Dihydroxypropyl-Methacrylat ist, Z das Polymerisationsradikal von Vinylsulfonat ist und z ein molarer Prozentanteil im Bereich von 1 bis 50 % ist.

8. Verfahren nach Anspruch 1, wobei X das Polymerisationsradikal von Acrylamid ist, Y das Polymerisationsradikal von 1,2-Dihydroxypropyl-Methacrylat ist, Z das Polymerisationsradikal von Vinylphosphonat ist und z ein molarer Prozentanteil im Bereich von 1 bis 50% ist.

9. Verfahren nach Anspruch 1, wobei X das Polymerisationsradikal von Acrylamid ist, Y das Polymerisationsradikal von Hydroxyethyl-Methacrylat ist, Z das Polymerisationsradikal von Vinylsulfonat ist und z ein molarer Prozentanteil im Bereich von 1 bis 50 % ist.

10. Verfahren nach Anspruch 1, wobei X das Polymerisationsradikal von Acrylamid ist, Y das Polymerisationsradikal von Hydroxyethyl-Methacrylat ist, Z das Polymerisationsradikal von Vinylphosphonat ist und z ein molarer Prozentanteil im Bereich von 1 bis 50 % ist.

11. Verfahren nach Anspruch 1, wobei X das Polymerisationsradikal von Acrylamid ist, Y das Polymerisationsradikal von 1,2-Dihydroxypropyl-Methacrylat ist, Z das Polymerisationsradikal von 2-acrylamido-2-methylpropan-Sulfonsäure ist und z ein molarer Prozentanteil im Bereich von 1 bis 50 ist.

12. Verfahren nach Anspruch 1, wobei X das Polymerisationsradikal von Acrylamid ist, Y das Polymerisationsradikal von Hydroxyethyl-Methacrylat ist, Z das Polymerisationsradikal von 2-acrylamido-2-methylpropan-Sulfonsäure ist und z ein molarer Prozentanteil im Bereich von 1 bis 50 % ist.

13. Verfahren nach Anspruch 1, wobei X das Polymerisationsradikal von Acrylamid und t-Butylacrylamid ist, Y das Polymerisationsradikal von 1,2-Dihydroxypropyl-Methacrylat ist und z = 0 ist.

14. Verfahren nach Anspruch 1, wobei X das Polymerisationsradikal von Acrylamid und Methacrylamid ist, Y das Polymerisationsradikal von 1,2-Dihydroxypropyl-Methacrylat ist und z = 0 ist.

15. Verfahren nach Anspruch 1, wobei X das Polymerisationsradikal von Acrylamid und Methacrylamid ist, Y das Polymerisationsradikal von Hydroxyethyl-Methacrylat ist und z = 0 ist.

16. Verfahren nach Anspruch 1, wobei Y eine glyoxylierte Acrylamideinheit darstellt und y kleiner als ungefähr 40 ist.

17. Verfahren nach Anspruch 1, wobei X das Polymerisationsradikal von Acrylamid und t-Butylacrylamid ist, Y das Polymerisationsradikal von Hydroxyethyl-Methacrylat ist und z = 0 ist.

18. Verfahren nach einem der vorigen Ansprüche, wobei das Polysaccharid Guar-Gummi ist.

19. Verfahren nach einem der Ansprüche 1-17, wobei das Polysaccharid Carboxymethyl-Zellulose ist.

20. Verfahren nach einem der Ansprüche 1-17, wobei das Polysaccharid Stärke ist.

## Revendications

1. Procédé pour enrichir des minéraux de valeur à base de sulfures provenant de minerais avec rejet sélectif de minéraux de gangue silicates non sulfurés, comprenant les étapes consistant à :
a. fournir une suspension de pulpe aqueuse de particules de minerai finement divisées d'une dimension appropriée à la libération qui contiennent lesdits minéraux de valeur à base de sulfures et lesdits minéraux de gangue silicates non sulfurés ;
b. conditionner ladite suspension de pulpe respectivement avec une quantité efficace de déprimant de minéraux de gangue silicates non sulfurés, un collecteur de minéraux de valeur à base de sulfures et un agent de moussage, ledit déprimant comprenant (1) un polymère ou un mélange de polymères comprenant :
(i) x motifs de formule :
⁅X⁆
(ii) y motifs de formule :
⁅Y⁆
(iii) z motifs de formule :
⁅Z⁆
dans lesquels X est le résidu de la polymérisation d'un monomère acrylamide ou d'un mélange de monomères acrylamides, Y est un motif polymère contenant un groupe hydroxy, Z est un motif polymère contenant un groupe anionique, x représente une fraction résiduelle en pourcentage molaire d'au moins 35%, y est une fraction en pourcentage molaire allant d'environ 1 à 50% et z est une fraction en pourcentage molaire allant de 0 à 50%, ou (2) un mélange dudit polymère ou desdits polymères et d'un polysaccharide, avec la condition que, dans le cas où l'on utilise un polyacrylamide glyoxylé comme déprimant, il contient moins de 50% en moles de motifs amides glyoxylés en tant que motif Y, et
c. recueillir le minéral de valeur à base de sulfure ayant une teneur réduite en minéraux de gangue silicates non sulfurés au moyen d'une flottation par moussage.

2. Procédé selon la revendication 1, dans lequel Y possède la formule dans laquelle A représente O ou NH, R et R¹ représentent, individuellement un atome d'hydrogène ou un groupe d'alkyle en C₁ à C₄ et n vaut de 1 à 3 inclus.

3. Procédé selon la revendication 1, dans lequel X est le résidu de polymérisation de l'acrylamide, Y est le résidu de polymérisation du méthacrylate de 1,2-dihydroxypropyle, et z vaut 0.

4. Procédé selon la revendication 1, dans lequel X est le résidu de polymérisation de l'acrylamide, Y est le résidu de polymérisation du méthacrylate de 1,2-dihydroxypropyle, Z est le résidu de polymérisation de l'acide acrylique et z est une fraction en pourcentage molaire allant de 1 à 50.

5. Procédé selon la revendication 1, dans lequel X est le résidu de polymérisation de l'acrylamide, Y est le résidu de polymérisation du méthacrylate d'hydroxyéthyle, et z vaut 0.

6. Procédé selon la revendication 1, dans lequel X est le résidu de polymérisation de l'acrylamide, Y est le résidu de polymérisation du méthacrylate d'hydroxyéthyle, Z est le résidu de polymérisation de l'acide acrylique et z est une fraction en pourcentage molaire allant de 1 à 50%.

7. Procédé selon la revendication 1, dans lequel X est le résidu de polymérisation de l'acrylamide, Y est le résidu de polymérisation du méthacrylate de 1,2-dihydroxypropyle, Z est le résidu de polymérisation du sulfonate de vinyle et z est une fraction en pourcentage molaire allant de 1 à 50%.

8. Procédé selon la revendication 1, dans lequel X est le résidu de polymérisation de l'acrylamide, Y est le résidu de polymérisation du méthacrylate de 1,2-dihydroxypropyle, Z est le résidu de polymérisation du phosphonate de vinyle et z est une fraction en pourcentage molaire allant de 1 à 50%.

9. Procédé selon la revendication 1, dans lequel X est le résidu de polymérisation de l'acrylamide, Y est le résidu de polymérisation du méthacrylate d'hydroxyéthyle, Z est le résidu de polymérisation du sulfonate de vinyle et z est une fraction en pourcentage molaire allant de 1 à 50%.

10. Procédé selon la revendication 1, dans lequel X est le résidu de polymérisation de l'acrylamide, Y est le résidu de polymérisation du méthacrylate d'hydroxyéthyle, Z est le résidu de polymérisation du phosphonate de vinyle et z est une fraction en pourcentage molaire allant de 1 à 50%.

11. Procédé selon la revendication 1, dans lequel X est le résidu de polymérisation de l'acrylamide, Y est le résidu de polymérisation du méthacrylate de 1,2-dihydroxypropyle, Z est le résidu de polymérisation de l'acide 2-acrylamido-2-méthylpropanesulfonique et z est une fraction en pourcentage molaire allant de 1 à 50%.

12. Procédé selon la revendication 1, dans lequel X est le résidu de polymérisation de l'acrylamide, Y est le résidu de polymérisation du méthacrylate d'hydroxyéthyle, Z est le résidu de polymérisation de l'acide 2-acrylamido-2-méthylpropanesulfonique et z est une fraction en pourcentage molaire allant de 1 à 50%.

13. Procédé selon la revendication 1, dans lequel X est le résidu de polymérisation de l'acrylamide et du t-butylacrylamide, Y est le résidu de polymérisation du méthacrylate de 1,2-dihydroxypropyle et z vaut 0.

14. Procédé selon la revendication 1, dans lequel X est le résidu de polymérisation de l'acrylamide et du méthacrylamide, Y est le résidu de polymérisation du méthacrylate de 1,2-dihydroxypropyle et z vaut 0.

15. Procédé selon la revendication 1, dans lequel X est le résidu de polymérisation de l'acrylamide et du méthacrylamide, Y est le résidu de polymérisation du méthacrylate d'hydroxyéthyle et z vaut 0.

16. Procédé selon la revendication 1, dans lequel Y représente un motif acrylamide glyoxylé et y est inférieur à environ 40.

17. Procédé selon la revendication 1, dans lequel X est le résidu de polymérisation de l'acrylamide et du t-butylacrylamide, Y est le résidu de polymérisation du méthacrylate d'hydroxyéthyle et z vaut 0.

18. Procédé selon l'une quelconque des revendications précédentes, dans lequel le polysaccharide est la gomme de guar.

19. Procédé selon l'une quelconque des revendications 1 à 17, dans lequel le polysaccharide est la carboxyméthylcellulose.

20. Procédé selon l'une quelconque des revendications 1 à 17, dans lequel le polysaccharide est l'amidon.
